

## UNITED STATES PATENT OFFICE.

CHARLES MCKNIGHT, JR., OF SEWICKLEY, PENNSYLVANIA, ASSIGNOR TO THE INTERNATIONAL NICKEL COMPANY, OF NEW YORK, N. Y., A CORPORATION OF NEW JERSEY.

## METHOD OF MAKING ALLOY STEELS.

No Drawing. Application filed June 8, 1925, Serial No. 35,788. Renewed March 13, 1928.

My invention relates to the making of alloy steel from ferrous materials which contain a considerable or large percentage of silicon.

The invention relates especially to the manufacture of alloy steels in the electric furnace, although within my broader claims, it may be used for any other methods of steel manufacture.

In the making of such alloy steels, especially in the electric furnace, manufacturers have had much difficulty in casting due to sudden and violent evolution of gases when the metal in the mold is near the solidification point. Many ingots have been scrapped on account of this wildness in the mold. This action has occurred intermittently and without known cause therefor. Powerful deoxidizers have been employed to overcome this trouble and various slags and temperatures have been tried to overcome it.

During the course of considerable research on this subject, I have discovered that the main cause for this inexplicable action has been the presence of silicon-bearing material in the charge from which the alloy steel is made. I have also discovered that this injurious action can be substantially done away with by reducing the silicon below .10%, and preferably below .05% during the working of the charge.

In the ordinary use of an electric furnace for making alloy steels, the charge is melted down under oxidizing influences with a black or "melt down" slag, after which this slag is removed and white or finishing slag fed to the bath and reducing conditions provided during the remainder of the heat. I have found that if, during the oxidizing period, the silicon is burnt out of the charge to reduce it to a point less than .10%, and preferably less than .05%, the difficulty above referred to is removed. Thereafter silicon may be added, if a normal or high silicon content is desired, without producing wildness or sudden rising of the metal in the mold.

I have also found that the same beneficial effect is obtained where chromium or nickel or both are added to the charge before casting. In the making of many if not all of these alloy steels, this same difficulty of wildness in the mold has occurred, and I have found it to be largely due to the fact that silicon was not sufficiently reduced in the

charge prior to the addition of the alloying metal or metalloid. 55

In carrying out my invention, the silicon may be removed by oxidizing it to silica in any desirable manner, preferably by boiling or exposing it to an oxidizing atmosphere, and also by adding oxides to the bath or using oxides in the charge. In any event, the silicon should be reduced to below .10% and preferably below .05%, after which the heat may be conducted in the usual manner to bring the bath to the desired analyses and to the quiescent state desirable to insure sound metal in the mold. 60 65

While the invention is especially desirable in the making of alloy steels in electric furnaces, it is also applicable to and highly desirable in the manufacture of alloy steels in other ways, as for example, in the open hearth. In all cases, the silicon should be reduced to the low point above referred to prior to the addition of the alloying ingredients, which 70 75 may be and preferably are added in the furnace prior to tapping.

The invention is especially desirable where the charge contains material having a considerable or large percentage of silicon, such 80 for example, as high silicon scrap, whether the scrap contains nickel or chromium or other alloying metal.

In the present manufacture of alloy steel, much of the scrap metal does contain considerable proportions of silicon, and I have discovered that if this silicon is not reduced below a critical percentage, the trouble with sudden rising or wildness of the steel in the mold occurs. 85 90

Many variations may be made in the method of making the steel, and other changes may be made without departing from my invention.

I claim: 95

1. The method of stabilizing the solidification of an alloy steel casting formed from scrap initially having a high silicon content, which consists in melting the metal under oxidizing conditions until the silicon content is below a critical point, wherein the silicon does not exceed .1%, subjecting the metal to a reducing condition and adding alloying materials thereto. 100

2. The method of stabilizing the solidification of an alloy steel casting formed from

scrap initially having a high silicon content, which consists in melting the metal under oxidizing conditions until the silicon content has been reduced to a point where it indicates 5 a satisfactory gas condition in the metal, thereafter treating the metal under a reducing condition, and adding alloying material.

3. The method of stabilizing the solidification of an alloy steel casting formed from 10 a charge initially having a high silicon content, which consists in melting the charge in an electric furnace under oxidizing conditions, reducing the silicon content to a point where a satisfactory gas condition in the 15 metal is indicated, thereafter treating the metal in a reducing atmosphere and adding alloying material.

4. The method of producing a casting having a high silicon content, which consists in 20 melting the charge in an electric furnace and exposing the same to an oxidizing atmosphere, reducing the silicon content to below .05%, thereafter subjecting the metal to a reducing condition and adding alloying materials, and casting the metal.

5. In the manufacture of substantially sound castings of alloy steel from ferrous charges having a silicon content considerably above .10% and also relatively high in metal 25 alloy content, the steps consisting of oxidizing the said charge in molten condition until silicon reduction to a point not exceeding

.10% indicating that troublesome gases are sufficiently eliminated, then working the heat until the proper conditions are attained, then 35 deoxidizing and then casting the refined material.

6. In the manufacture of substantially sound castings of alloy steel from ferrous charges having a silicon content considerably 40 above .10% and also relatively high in metal alloy content, the steps consisting of oxidizing the said charge in molten condition until silicon reduction to a point not exceeding .05% indicating that troublesome gases are 45 sufficiently eliminated, then working the heat until the proper conditions are attained, then deoxidizing and then casting the refined material.

7. In the manufacture of substantially sound castings of alloy steel from ferrous charges having a silicon content considerably 50 above .10% and also relatively high in metal alloy content, the steps consisting of oxidizing the said charge in molten condition until silicon reduction to a point not exceeding .10% indicating that troublesome gases are 55 sufficiently eliminated, then working the heat until the proper conditions are attained, then adding alloy material and deoxidizing, and 60 then casting the refined material.

In testimony whereof I have hereunto set my hand.

CHARLES McKNIGHT, JR.